

Dec. 22, 1953

L. SCHLECHT ET AL

2,663,630

PRODUCTION OF METAL POWDERS

Filed Oct. 21, 1950



INVENTORS:  
LEO SCHLECHT  
ERNST OESTREICHER

BY *Spencer, Johnston,  
Cook & Root*

ATT'YS

## UNITED STATES PATENT OFFICE

2,663,630

## PRODUCTION OF METAL POWDERS

Leo Schlecht and Ernst Oestreicher, Ludwigshafen (Rhine), Germany, assignors to Badische Anilin- & Soda-Fabrik Aktiengesellschaft, Ludwigshafen (Rhine), Rheinland - Pfalz, Bundesrepublik, Germany

Application October 21, 1950, Serial No. 191,500

Claims priority, application Germany  
November 4, 1949

4 Claims. (Cl. 75—0.5)

1

This invention relates to improvements in the production of metal powders by thermal decomposition of metal carbonyls.

In carrying out this known process, the metal carbonyls, preferably in the vapor phase, are led into a chamber which is externally heated to temperatures above the decomposition temperature of the carbonyl, the decomposition of the carbonyl taking place in the hot free space of the chamber substantially at a distance from the hot walls of the chamber. In this way there is generally obtained a metal powder of high purity and some carbon-content which is composed of particles of different sizes. Since, however, for many purposes a definite size of particles is desired, attempts have been made to separate the undesirable particles from the powder by subsequently subjecting the powder to a wind sifting. During the withdrawal of the powder from the decomposition chamber and its conveyance into the wind sifting plant, loosely agglomerated powder particles which usually deposit on the walls of the decomposition chamber and which have a higher carbon content than the individual, non-agglomerated particles, are in part triturated so that in the subsequent wind sifting these particles with higher carbon content also pass into the fraction obtained by sifting and injuriously affect the uniformity of this fraction.

We have now found that the said drawback can be avoided by leading through the decomposition chamber, during or after the decomposition of the metal carbonyl, a current of gases or vapors, preferably a current of carbon monoxide, and recovering the metal powder entrained by the gases leaving the decomposition chamber. In this way it is possible to retain the original form of the agglomerates of the elementary particles and to recover these structures, which are usually in the form of small sponges or tufts, separately from the non-agglomerated particles of the powder. The separation from the gases may be effected in a plurality of stages, for example by means of several, consecutively arranged filters, deflecting or baffle plates or the like, and in this way a plurality of fractions of particles of definite sizes may be obtained.

The simplest procedure is to carry out the carbonyl decomposition in an elongated cylindrical container arranged vertically, and to lead in the gases axially at the bottom of the container. By providing a conical cover over the opening of the upwardly directed inlet pipe a desired direction, for example obliquely downwards, can be imparted to the current of gas.

2

The degree of separation and sifting of the metal powder can be influenced by the amount of gas led in. When it is desired to separate from the powder only the finest particles, a smaller amount is generally employed. If, on the other hand, it is important to separate the coarsest particles from the powder, the bulk of the powder is blown from the decomposition chamber, by means of a powerful current of gas introduced at the bottom of the decomposition chamber, into the adjacent separation or sifting apparatus.

The gases may be led in at such a low temperature that they effect a cooling of the metal powder and carbon monoxide formed by the decomposition. In this case care should be taken that the carbonyl is already completely decomposed before the cold gas is led in. By the said cooling there is the advantage that undesirable decomposition of the carbon monoxide, which causes an enrichment of carbon in the metal powder, is minimised.

An apparatus suitable for carrying out the process of the invention is schematically represented in the accompanying drawing. In the drawing, a vertically arranged generally cylindrical container 1 is provided with a carbonyl vapor inlet tube 2 at its top and heating means 3 externally surrounding its side. The bottom of the container 1 is constructed to provide conical portions 4 and 5, and the lower conical portion 5 is provided with a valve 6 or the like, through which metal powder is withdrawn.

A gas inlet tube 7 leading from a source of gas, such as carbon monoxide, enters the bottom section of the container 1 through the wall of the upper conical portion 4 and extends to the axis of the container, where it is turned upwardly, in line with the axis. Spaced above the open end of the gas inlet tube 7 within the container and adjacent the tube end is a conical cover 8, arranged with its apex pointing upwardly, to deflect the gas entering through the tube 7 obliquely downwards.

A gas exit tube 9 is connected to the upper conical portion 4 of the container 1 and communicates with the interior of the container. The exit tube 9 is connected at its other end to a separator 10, which includes a vertically arranged cylindrical collecting chamber 11, a valve 12 or the like at the lower end of the chamber 11 through which metal powder is withdrawn, an enlarged chamber 13 at the upper end of the collecting chamber 11 which encloses a filter 14, and a filtered gas exit tube 15 at the upper end of the enlarged chamber 13.

In operation according to the above-described

procedures, metal carbonyl vapor is passed through the vapor inlet tube 2 and into the container 1, maintained above the decomposition temperature of the carbonyl by the heating means 3. As decomposition progresses, metal powder forms and falls and is carried downwardly in the container 1.

During or after the decomposition of the carbonyl vapor, gas such as carbon monoxide is passed into the container 1, through the gas inlet tube 7. The gas is deflected by the cover 8 obliquely downwardly, so that the gas traverses the container 1. In so doing, part of the metal powder coming down in the container is entrained in the gas. The gas and entrained powder leave the container through the exit tube 9 and pass into the separator 10. In the separator, powder is removed from the gas by the filter 14 and is collected in the collecting chamber 11, from which it is withdrawn as desired through the valve 12. The filtered gas leaves the separator through the exit tube 15. Meanwhile, coarser metal powder which is not entrained in the gas collects in the lower conical portion 5 of the container 1, from which it is removed through the valve 6.

The following example will further illustrate the invention but the invention is not limited to this example.

*Example*

In the decomposition of iron carbonyl with an addition of some ammonia in an externally heated cylindrical container having an internal diameter of 1 metre and a height of 5 metres. 56% of the total amount of iron powder formed by the decomposition separate at the bottom of the container while the remaining 44% are entrained into an adjacent laterally arranged filter by the carbon monoxide formed by the decomposition and leaving the container. The iron powder withdrawn from the bottom of the decomposition container contains 0.83% of carbon and that collected in the filter contains 0.59% of carbon. By wind sifting of the powder withdrawn from the bottom in a current of nitrogen, a finest fraction is obtained having a carbon content of 0.62%.

If, on the other hand, in the same decomposition container operated under the same conditions, carbon monoxide is led in axially at the bottom, the fraction of powder in the laterally arranged filter is increased from 44% to 58% with the same carbon content of 0.59%. In this way the proportion of iron powder with the lowest carbon content is increased by about 30%.

What we claim is:

1. In the process of producing metal powders by thermal decomposition of metal carbonyls in the hot free space of an elongated vertical cylindrical container the step which comprises separating a fraction of powder characterized by low carbon content by leading a current of gas through the said container while introducing the gas axially at the bottom and imparting

to the gas current an obliquely downward direction, so as to entrain a portion of the metal powder formed in said free space, leading said current of gas out of said container to a solids separator, and separating from the gas the metal powder entrained by the current.

2. In the process of producing metal powders by thermal decomposition of metal carbonyls in the hot free space of an elongated vertical cylindrical container the step which comprises separating a fraction of powder characterized by low carbon content by leading a current of carbon monoxide gas through the said container while introducing the gas axially at the bottom and imparting to the gas current an obliquely downward direction, so as to entrain a portion of the metal powder formed in said free space, leading said current of gas out of said container to a solids separator, and separating from the gas the metal powder entrained by the current.

3. In the process of producing metal powders by thermal decomposition of metal carbonyls in the hot free space of a heated container the step which comprises separating a fraction of powder characterized by low carbon content by leading a current of gas through the container at such a temperature that a simultaneous cooling of the metal powder and carbon monoxide formed by the decomposition is effected, while introducing the gas axially at the bottom and imparting to the gas current an obliquely downward direction, so as to entrain a portion of the metal powder formed in said free space, leading said current of gas out of said container to a solids separator, and separating from the gas the metal powder entrained by the current.

4. In the process of producing metal powders by thermal decomposition of metal carbonyls in the hot free space of an elongated vertical cylindrical container the step which comprises separating a fraction of powder characterized by low carbon content by leading a current of carbon monoxide through the said container axially from its bottom at such a temperature that a simultaneous cooling of the metal powder and carbon monoxide formed by the decomposition is effected, while imparting to the gas current an obliquely downward direction, so as to entrain a portion of the metal powder formed in said free space, leading said current of gas out of said container to a solids separator, and separating from the gas the metal powder entrained by the current.

55 LEO SCHLECHT.  
ERNST OESTREICHER.

References Cited in the file of this patent

UNITED STATES PATENTS

| Number    | Name            | Date           |
|-----------|-----------------|----------------|
| 1,836,732 | Schlecht et al. | Dec. 15, 1931  |
| 1,877,861 | Hatch           | Sept. 20, 1932 |
| 1,893,913 | Saint-Jacques   | Jan. 10, 1933  |
| 2,389,701 | Truesdale       | Nov. 27, 1945  |
| 2,460,546 | Stephanoff      | Feb. 1, 1949   |